

# UNITED STATES PATENT OFFICE.

PASCAL MARINO, OF LONDON, ENGLAND.

## ELECTROLYTIC PROCESS FOR REMOVING OXID OR RUST.

1,195,704.

Specification of Letters Patent. Patented Aug. 22, 1916.

No Drawing.

Application filed April 25, 1916. Serial No. 93,392.

*To all whom it may concern:*

Be it known that I, PASCAL MARINO, a subject of the King of Italy, and resident of 19 St. Mary's Terrace, Harrow Road, 5 London, England, have invented an Electrolytic Process for Removing Oxid or Rust, of which the following is a specification.

This invention consists in a process whereby oxid or rust which has been formed on an 10 iron or steel surface may be removed.

According to this invention the article is employed as a cathode in an aqueous bath either of phosphoric acid or of a phosphoric acid compound to which phosphoric acid 15 has been added. The electrolyte is constituted either by a solution of ten parts of phosphoric acid in ninety parts of water or by an aqueous solution of a phosphoric acid compound to which has been added ten per 20 cent. of phosphoric acid *e. g.* to a 10% aqueous solution of sodium phosphate is added ten per cent. of concentrated phosphoric acid. As is well known the conductivity of liquids increases with their temperature. Consequently in order to allow 25 the electric current to act more efficiently and to detach and remove the layer of oxid or rust more rapidly the temperature of the electrolyte should be raised until it attains 30 50° to 70° C. so that the electro-chemical action may take place more readily. Conductive plates of carbonaceous material or lead are placed in the electrolyte and serve 35 as anodes, the articles treated when immersed in the bath serving as cathodes. The effect of the electric current is to remove the layer of oxid from the article under treatment with the result that its surface becomes quite clean and ready for any subsequent 40 technical or electro-chemical operation.

By the use of the word "iron" in the claims, I do not intend to limit my invention, but on the contrary, intend it to include steel as an equivalent thereof. Where in the claims I speak of "an aqueous bath containing phosphoric acid" I mean a bath which does not contain any material or compound that, under the action of the electric current, will cause a deposit to be formed upon the article used as a cathode. 45

Having now particularly described and ascertained the nature of my said invention and in what manner the same is to be performed, I declare that what I claim is:—

1. The process of electrolytically removing oxid from the surface of iron articles which comprises employing such articles as cathodes in an aqueous bath containing phosphoric acid. 55

2. The process of electrolytically removing oxid from the surface of iron articles which comprises employing such articles as cathodes in an aqueous bath containing a phosphoric acid compound and phosphoric acid. 60

3. The process of electrolytically removing oxid from the surface of iron articles which comprises employing such articles as cathodes in an aqueous bath of a phosphoric acid compound which contains 10 per cent. of concentrated phosphoric acid. 70

4. The process of electrolytically removing oxid from the surface of iron articles which comprises employing such articles as cathodes in an aqueous bath containing 10 per cent. of concentrated phosphoric acid. 75

Dated this 7th day of April 1916.

PASCAL MARINO.